

1

3,498,856  
COMBUSTION CATALYST FOR SOLID AMMONIUM NITRATE PROPELLANT GRAINSamuel W. Harris, Chicago, Ill., assignor to Standard Oil Company, Chicago, Ill., a corporation of Indiana  
No Drawing. Filed July 24, 1967, Ser. No. 655,328  
Int. Cl. C06d 1/00

U.S. Cl. 149—19

5 Claims

## ABSTRACT OF THE DISCLOSURE

Propellant grain containing a major amount of ammonium nitrate as the primary oxidizer, polymeric olefin as the primary binder and an effective amount of combustion catalyst comprising a hydrocarbon having a boiling point of between 150° C. and 500° C. and which is capable of forming a peroxide at a temperature in the range of the combustion of the propellant.

## BACKGROUND OF THE INVENTION

This invention relates to a new class of propellant compositions more particularly to ammonium nitrate compositions having a polymeric olefin binder and a novel combustion catalyst.

Ammonium nitrate is classified as a high explosive even though it is extremely insensitive and cannot be readily ignited by the local application of heat or by a blasting cap. Even when ignited, ammonium nitrate alone does not consistently sustain the propagation of combustion. In order to utilize the excess oxygen available from the decomposition of ammonium nitrate, oxidizable materials are mixed with the ammonium nitrate. Generally, these mixtures of ammonium nitrate and oxidizable material are more sensitive than the ammonium nitrate alone, but the mixtures are also insensitive and slow burning. The utilization of certain binder materials, which provide excellent stability and good ballistic properties, generally create even more insensitive compositions due to the stability. Such a class of binder systems, as for example, polymeric olefins, e.g. polyethylene, and polyethylene derivatives, are highly desirable, but in certain applications, it is necessary to incorporate into the composition a combustion catalyst which offers control of the burn rate.

One requirement for a solid propellant suitable for military use is that it be ballistically stable after long periods of storage at temperatures as high as 160° F. and as low as —65° F. Another requirement is that the burning of the composition following storage at either of these extremes, be uniform and not changed materially from the burning characteristics of such composition which has not been subjected to these conditions. The proper choice of a combustion catalyst, therefore, requires a consideration of the ability of the catalyst to aid in combustion only when called upon to do so. For this reason, it is necessary for the catalyst to be stable at all temperatures common to these storage conditions, but readily active at the initiation of combustion upon ignition.

## SUMMARY OF THE INVENTION

I have now discovered a novel catalyst system which meets all the requirements set forth above, and which is useful in ammonium nitrate containing solid propellants having a stable polyolefin binder. The catalyst system comprises hydrocarbon-containing compounds which readily form peroxides at a temperature in the range of the combustion temperature. It is understood that the compositions of the present invention may also contain various other additives such as carbon, stabilizers, etc.

The term "ammonium nitrate" as used in this specifi-

2

tion and in the claims is intended to mean either ordinary commercial grade ammonium nitrates such as conventionally grained ammonium nitrate containing a small amount of impurities which may be coated with a small amount of moisture-resisting material such as petrolatum or paraffin, or to mean military grade ammonium nitrate or mixture of minor amounts (usually less than 10%) of other organic or inorganic nitrates such as guanidine nitrate or sodium nitrate or potassium nitrate with the ammonium nitrate in a mixture of finely ground and unground or coarsely ground ammonium nitrate is preferred. The major proportion of the ammonium nitrate should be finely ground, but it is well known in the propellant art that particle size and size distribution within the composition are related to the ballistic properties. The amount of grinding then, will depend upon the desired properties of the propellant.

The polyolefin binder material may be any polymeric olefin known to the art as a binder material for use in ammonium nitrate based solid propellants, for example, polyethylene; Surlyn A type polymers (which is the subject of copending application, S.N. 655,300 filed July 24, 1967); etc. The Surlyn A compositions may be obtained commercially from E. I. du Pont de Nemours and Company.

The combustion catalyst is a hydrocarbon-containing compound having at least one active site capable of forming a peroxide radical at temperatures in the range of the combustion of the composition into which the catalyst is incorporated. Substantially all active sites are reacted at said temperature. However, the catalyst should be stable, i.e. exhibit substantially no peroxide formation, at temperatures to which the grain is subjected during storage. It is preferred that the active site be capable of oxidation to form the peroxide radical. The catalyst, therefore, should undergo substantially complete oxidation to form peroxide at a temperature in the range of approximately 125° C. to 250° C., and substantially no oxidation below about 125° C. The catalyst must have a boiling point in the range of 150° C. to 500° C., in order to provide the desired volatility. It is preferred that the catalyst contain tertiary hydrogen, since these compounds are known to readily form peroxides. Exemplary of the compounds suitable for use in this invention are partially hydrogenated naphthalenes, e.g. tetrahydronaphthalene; partially hydrogenated anthracenes, e.g. octahydroanthracene; cumene; substituted cumenes, e.g. phenylcumene; polybutene containing tertiary hydrogen and having a molecular weight above 300, preferably in the range of 300 to 2,000; etc. The compounds suitable in this invention may also contain atoms other than carbon and hydrogen, for example, nitrogen and nitrogen-containing groups.

It is also desired that the composition contain a carbon component. The finely divided carbon may be added in amounts up to 10% by weight of the composition, preferably in amounts of 1 to 5% by weight for the purpose of improving the burning rate of the composition. Highly adsorptive activated carbons such as "Norite" and "Nuchar" well known in the art as activated carbon of vegetable origin, make up one class of effective burning rate components. A second general class of carbon useful for increasing the burning rate of compositions are the carbon blacks, roughly classified as the channel blacks and the furnace combustion blacks. The carbon blacks are characterized by low ash content, that is, less than about 0.5%, usually less than about 0.15%, and by having extremely small particle size, that is 50 to 5,000 Å. and contain adsorbed hydrogen and oxygen. "Bead" type carbon blacks, such as Micronex Beads and Statex Beads, are also suitable. A third type of carbon which may be used is finely ground petroleum coke, particularly petro-

leum coke obtained as residue in the pipe-stilling of mid-continent heavy residuums.

The oxidizer and binder should be present in the composition in essentially stoichiometric amounts, in order to best utilize the excess oxygen obtained from the oxidizer, and an effective amount of catalyst must be present. A major amount of oxidizer should be present. Suitable propellant compositions comprise:

|                                                            | Percent by weight |
|------------------------------------------------------------|-------------------|
| (a) Binder                                                 | 5 to 40           |
| (b) Catalyst                                               | 0.5 to 5          |
| (c) Carbon                                                 | 0 to 10           |
| (d) Remainder of composition essentially ammonium nitrate. |                   |

Preferred compositions are as follow:

|                                                            | Percent by weight |
|------------------------------------------------------------|-------------------|
| (a) Binder                                                 | 15 to 30          |
| (b) Catalyst                                               | 1.5 to 3.5        |
| (c) Carbon                                                 | 1 to 5            |
| (d) Remainder of composition essentially ammonium nitrate. |                   |

Other additives which may be added are present in an amount sufficient to provide effective improvement of the properties for which they are added.

In preparing the compositions of this invention, any procedure known to the art for the preparation of ammonium nitrate grains containing a thermoplastic binder may be used.

With respect to the properties of a solid propellant, the velocity at which a solid propellant is consumed during operation is called the burning rate. It is measured in a direction normal to the propellant surface and is usually expressed in inches per second. The burning rate may be expressed by the following relation, in which the influence of all performance parameters is small compared to the chamber pressure and the initial grain temperature.

$$r = ap^n$$

The burning rate or velocity of propellant consumption "r" is usually given in inches per second; the chamber pressure "p<sub>c</sub>" in pounds per square inch; "a" and "n" are constants. The constant "a" varies with the initial propellant temperature, and thus the burning rate is a function of the temperature of the grain prior to combustion. The lower the value of "n," the less is the detonating character of the decomposition of a gas producing composition and the more even and smooth is the burning rate of the propellant grain. Thus, a sustained thrust rather than a detonation is obtained by smooth burning of the grain.

The temperature sensitivity for different solid propellants is usually expressed as the percentage change of thrust per unit of temperature change. Temperature changes effect the equilibrium pressure and the burning rate. The definitions of the temperature coefficients are given by Sutton, "Rocket Propulsion Elements" (2nd ed. 1958).

$$\pi_K = \frac{(\delta \ln p)}{(\delta T)_K} = \frac{1}{P_c} \frac{(\delta P)}{(\delta T)_K}$$

$$\sigma_p = \frac{(\delta \ln r)}{(\delta T)_p} = \frac{1}{r} \frac{(\delta r)}{(\delta R)_p}$$

Here  $\pi_K$  is the temperature sensitivity coefficient of equilibrium pressure at a particular value of K (K is the ratio of the burning surface to the throat area), expressed in percent pressure change per degree temperature change. Mathematically it is defined as the partial derivative of the natural logarithm of the equilibrium chamber pressure  $p$  with respect to temperature  $T$ . The other temperature sensitivity coefficient  $\sigma_p$  refers to the change in burning rate  $r$  of a solid propellant with respect to temperature  $T$  at a particular value of chamber pressure  $p_c$ . It is also known as the burning rate temperature coefficient, while  $\pi_K$  is known as the temperature sensitivity of pressure.

For most propellant applications, as low a temperature coefficient as possible is desirable and even required for engineering design consideration. Lower pressure levels over a given temperature level allows a sizable weight savings for most missile applications.

#### DESCRIPTION OF PREFERRED EMBODIMENTS

The following examples are given by way of illustration and should not be construed as limiting.

Examples 1-6 of the following procedure was used in producing the propellant grains identified in the examples: The ingredients were mixed in a sigma blade mixer using a 110° C. jacket temperature, until the mixture was a plastic mass. The compositions are as follows:

| Example | Formulation         | Weight Percent |
|---------|---------------------|----------------|
| I       | Ammonium nitrate    | 73.0           |
|         | Carbon black        | 5.0            |
|         | Surlyn A            | 20.0           |
|         | Tetralin and cumene | 2.0            |
| II      | Ammonium nitrate    | 78.0           |
|         | Carbon black        | 3.0            |
|         | Surlyn A            | 17.0           |
|         | Octahydroanthracene | 2.0            |
| III     | Ammonium nitrate    | 78.0           |
|         | Carbon black        | 3.0            |
|         | Surlyn A            | 17.0           |
|         | Phenylecumene       | 2.0            |
| IV      | Ammonium nitrate    | 78.0           |
|         | Carbon black        | 3.0            |
|         | Polyethylene        | 17.0           |
|         | Octahydroanthracene | 2.0            |
| V       | Ammonium nitrate    | 78.0           |
|         | Carbon black        | 3.0            |
|         | Surlyn A            | 17.0           |
|         | Tetralin            | 2.0            |
| VI      | Ammonium nitrate    | 78.0           |
|         | Carbon black        | 3.0            |
|         | Surlyn A            | 17.0           |
|         | Cumene              | 2.0            |

The Surlyn A of the above formulations have a softening point of about 95° C., and contain sodium as the primary metallic ion. All of the above formulations were molded into grains and cut into strands for testing in a Crawford bomb. The results of the tests are shown in the table below.

TABLE

| Product of Example | Ballistic Properties |            |         |                       |
|--------------------|----------------------|------------|---------|-----------------------|
|                    | n                    | $\sigma_p$ | $\pi_K$ | $r_{1000}$ (in./sec.) |
| I                  | 0.45                 | 0.135      | 0.25    | 0.031                 |
| II                 | 0.55                 | 0.112      | 0.25    | 0.044                 |
| III                | 0.34                 | 0.112      | 0.17    | 0.034                 |
| IV                 | 0.94                 | 0.23       | -----   | 0.028                 |
| V                  | 0.75                 | 0.0826     | 0.33    | 0.034                 |
| VI                 | 0.64                 | 0.172      | 0.48    | 0.038                 |

What is claimed is:

1. A propellant composition comprising:
  - (a) a major amount of ammonium nitrate;
  - (b) a binder selected from the class consisting of polyethylene, and a polymeric material having a softening point in the range of from 80° C. to 120° C., said polymeric material comprising a crossed-linked thermoplastic resin containing:
    - (i) a major amount of ethylene units; and
    - (ii) interchain forces developed between carboxyl groups pendant from an alpha olefin chain and metallic ions selected from the group consisting of sodium, potassium, calcium, magnesium, and zinc; and
  - (c) from 0.5 to 5.0 weight percent of a combustion catalyst selected from the class consisting of partially hydrogenated naphthalenes, partially hydrogenated anthracenes, cumene, substituted cumenes, polybutenes containing tertiary hydrogen and having a molecular weight greater than 300.

2. The composition of claim 1 wherein said binder is present in the range of 5 to 40 weight percent; said catalyst is present in the range of 0.5 to 5.0 weight percent; carbon is present in the range of 0 to 10 weight percent; and the remainder of said composition is essentially ammonium nitrate.

3. The composition of claim 1 wherein said catalyst is tetrahydronaphthalene.

4. The composition of claim 1 wherein said catalyst is octahydroanthracene.

5. The composition of claim 1 wherein said catalyst is phenylcumene.

## References Cited

## UNITED STATES PATENTS

|             |        |                    |          |
|-------------|--------|--------------------|----------|
| 3,147,161   | 9/1964 | Abere et al. ----- | 149—19   |
| 3,305,523   | 2/1967 | Burnside -----     | 149—19 X |
| 5 3,338,764 | 8/1967 | Evans -----        | 149—19   |

BENJAMIN R. PADGETT, Primary Examiner

U.S. CL. X.R.

10 149—20